

Sept. 2, 1930.

G. K. WILLIAMS

1,774,688

REFINING OF LEAD BULLION

Filed March 28, 1929

high grade CRUSTS to refinery



Fig. 1.



Fig. 2.

Inventor

George K. Williams

by Spear, Middleton, Donaldson Hall  
Atty's.

## UNITED STATES PATENT OFFICE

GEORGE KENNETH WILLIAMS, OF PORT PIRIE, SOUTH AUSTRALIA, AUSTRALIA

## REFINING OF LEAD BULLION

Application filed March 28, 1929, Serial No. 350,832, and in Australia April 11, 1928.

This invention relates to the refining of lead bullion containing other metals such as copper, gold and silver, and refers more especially to the refining of bullion working under similar conditions to what is known as the "Parkes" process, that is to say, wherein zinc is added for the formation of alloys in the form of crusts.

For the purpose of avoiding unnecessary repetition in this specification the following terms will have the following meaning:

"Alloying metals" will mean such metals as copper or gold or silver which form alloys with zinc (with or without lead) and which being present in the initial bullion, it is desired to remove, both for their own values and for the purpose of providing lead sufficiently free therefrom for commercial purposes.

20 "Crusts" will mean and include alloys of the said alloying metals in the form of crusts which are formed by the cooling of the bullion with a view to separation from the lead bullion.

25 "Residual bullion" will mean the bullion remaining after one or more of the alloying metals has been separated therefrom in the form of crusts and is relatively low in such alloying metal or metals.

30 In the refining of lead bullion by the well-known "Parkes" process, it is the practice to incorporate a certain amount of zinc with the molten bullion sufficient for the formation of certain alloys of the alloying metals desired to be removed. The bullion is then cooled, whereby the said alloys separate from the bullion in the form of crusts, which, owing to their specific gravity being lower than that of the liquid bullion, rise to the surface and are then removed, leaving residual bullion relatively low in such alloying metals.

35 The crusts obtained by the aforesaid Parkes process contain a considerable amount of entangled lead, the removal of which has been effected either by subjecting the said crusts to liquation, or to presses.

According to a patent in the United States of America which has been granted to me No. 1,687,187, the treatment for the refining 45 of bullion is effected by incorporating zinc

with the said bullion in sufficient quantity and maintaining such temperatures that molten layers of conjugate solutions are formed, the upper of which consists of an alloy rich in certain alloying metal or metals and separating such alloy. In the operation of this process it has been applied to effect a continuous refining of lead bullion, by continuously feeding the molten bullion into a vessel and continuously withdrawing the residual bullion from the bottom thereof, and continuously or intermittently removing the alloy rich in certain alloying metal or metals from the top.

55 It has hitherto not been possible to effect a continuous refining of lead bullion by the Parkes process by reason of the fact that it is necessary to add the requisite quantity of zinc, and to heat the bullion for effecting the solution thereof in the lead, and to then cool the mass whereby the alloys are separated out as crusts. The nature of this operation has 60 hitherto necessitated the carrying out of this said Parkes process as an intermittent or batch treatment operation.

65 Now, the object of this invention is to provide a method of operation whereby the essential conditions and characteristics of the Parkes process may be obtained in a continuous operation as distinct from, on the one hand the intermittent or batch treatment at 70 present practised, and on the other hand from the formation of conjugate solutions as described in the aforesaid Patent No. 1,687,187.

75 I accomplish this object by incorporating with the bullion an amount of zinc governed by the content of alloying metals in the initial bullion on the one hand and in the residual bullion on the other hand and subjecting the said bullion during its continuous flow to a decreasing range of temperatures, the upper of which is sufficiently high for the solution of the zinc in the bullion and below the melting point of the alloy comprising the crusts to be removed, whilst the lower of such range is just above the eutectic temperature of the residual bullion desired to be produced, continuously withdrawing the residual bullion and continuously or intermittently removing the crusts accumulating.

80 The amount of zinc incorporated with the

bullion is, as stated, governed by the content of the alloying metals in the initial bullion and in the residual bullion, and in determining the amount of zinc additions necessary 5 regard will be had to the alloys which are formed in the cooler zones and which are re-dissolved in the bullion in the zones of higher temperature.

The refining operation is carried out in one 10 or more stages the essential feature of the invention being the continuous flow of the bullion through each stage. In practice each stage is represented by the flow of the bullion through a kettle or series of kettles or other 15 suitable vessel in which the zinc is incorporated with the bullion and the same subjected to the necessary decreasing range of temperatures. In normal practice of the Parkes process a stage is generally equivalent to what 20 is known as a "zincing". The invention however may be carried out in other suitable apparatus such as reverberatory furnaces in which the bullion may be subjected to the necessary decreasing range of temperature.

25 In the drawings:

Figure 1 is a view in sectional elevational of a series of two externally heated kettles adapted for carrying out the invention; and

Figure 2 is a diagrammatic view in elevation illustrating an alternative arrangement of apparatus, and hereinafter is fully described.

In carrying out this invention the molten bullion is preferably fed into the top of a 30 suitable kettle (see Fig. 1 of the drawings) where the requisite quantity of zinc necessary for the later formation of alloys in the form of crusts is incorporated with the bullion the temperature being at the upper part 35 of the said kettle sufficiently high for the incorporation in the bullion of the requisite quantity of zinc, but below, the melting point of the alloys comprising the said crusts, whilst the temperature at the bottom of the 40 kettle is maintained just above the eutectic temperature of the residual bullion, and continuously withdrawing the said residual bullion from the bottom of the kettle, and continuously or intermittently removing the 45 crusts from the top of the said kettle.

The shape and dimensions of the kettle in which the operation is conducted may be as shown in Fig. 1 and are such that the bullion in passing therethrough at a certain rate of 50 flow is subject to decreasing temperatures within the limits mentioned and for this purpose the kettles are so mounted in the brick-work that independent flues E and F surround the same so that differential temperatures may be applied thereto by suitable means.

In practice the bullion may be pre-heated to any desired temperature before being fed into the top of the kettle such as by means of 55 suitable reverberatory furnaces (Figure 2).

The necessary amount of zinc is incorporated with or dissolved in the molten bullion at the top of the kettle either in the form of virgin zinc in solid or liquid condition, or in the form of crusts obtained from a previous operation. In practice this zinc is supplemented by the formation of alloys in the form of crusts in the cooler zones which are re-disolved in the bullion in the hotter zones.

As the bullion passes downward through 75 the kettle into the cooler zones, crusts are formed which rise to the upper part of the kettle, whilst the residual bullion is continuously withdrawn from the bottom of the kettle in molten condition, either by being 80 pumped or siphoned, or overflowing therefrom through a suitable spout such as A<sup>1</sup> which discharges from the bottom and delivers just below the surface of the bullion. The crusts accumulating on the surface are 85 removed, either continuously or intermittently by manual or mechanical means as may be desired.

As with the Parkes process this invention is applicable to the treatment of bullion for 90 the differential separation of alloying metals or for the collective separation thereof. For example, the operation may be conducted by first obtaining crusts rich in one alloying metal, such as gold, followed by a subsequent 95 separation of crusts rich in another alloy, such as silver, or alternatively crusts may be obtained rich in two or more alloying metals, such as gold and silver.

Instead of conducting the operation in one 100 kettle, in which the residual bullion is withdrawn just above its eutectic temperature, the operation may be conducted in two or more kettles in series in which case it would only be necessary that the temperature should be 105 maintained just above the eutectic temperature of the residual bullion at the outflow from the last kettle of the series, though it will be understood that the operation may also be conducted with the temperature at 110 the bottom of all of the kettles in the series just above the eutectic temperature of the residual bullion.

The operation of the Parkes process at present practised is the subject of a number 115 of different well known modifications involving mostly the different points at which the additions of zinc are made, and this invention is applicable to any of the said modifications, the essential point being that the 120 cooling of the bullion for the formation of crusts is effected during the continuous passage of the bullion as distinct from the intermittent or batch treatment which has hitherto been incidental to the operation of the 125 said Parkes process. For example the invention is applicable to the well known modification of the Parkes process in which two successive zincings are employed, the necessary zinc for the first zincting being obtained 130

from crusts produced from the second zincing of a previous operation whilst virgin zinc is used for the second zincing.

In applying this invention to this modification of the Parkes process, it is desirable to make use of two kettles as shown in Fig. 5 1 in series, the outflow from kettle A being delivered into the top of kettle B. The crude bullion is continuously fed into the top of kettle A, preferably having been preheated 10 to a temperature sufficient for the incorporation of the requisite amount of zinc in the form of crusts, and below the melting point of the crusts which it is desired to remove from the top of this first kettle. This pre-heating may be effected in a suitable reverberatory furnace C as shown in Figure 2.

The crusts skimmed off from the top of kettle B are regularly delivered into the top 20 of kettle A with the feed of molten crude bullion. The temperature is maintained in the bottom of kettle A at just above the eutectic temperature of the residual bullion being delivered from kettle A and is governed by the grade of the metal which it is 25 desired to deliver to kettle B. The bullion outflows from A kettle into kettle B and virgin zinc is regularly supplied to the top of this kettle B in such quantities as are 30 necessary for the formation of the alloys with the alloying metals contained in the crude bullion. The top of kettle B is maintained at a temperature sufficiently high to ensure the incorporation in the bullion of the zinc 35 to be added, but below the melting point of the crusts formed in the said kettle B. In practice the temperatures at the top of both kettles are approximately the same. The bottom of kettle B is maintained at the temperature just above the eutectic temperature 40 of the residual bullion, which continuously outflows therefrom.

In operation these two kettles are working 45 in series in the same manner as obtains with the Parkes process, kettle A being directed to the formation of crusts of as high a grade as is possible in alloying metals, whilst the kettle B is directed towards the production 50 of a residual bullion of as low a content of alloying metals as is practicable.

In another application of this invention 55 operating in two kettles working in series, the virgin zinc requisite for the formation of the alloys with the alloying metals contained in the crude bullion may be added to kettle A as well as the crusts obtained from kettle B. In this case it will be necessary to maintain a higher temperature in the top of kettle A than in the previous example in view 60 of the higher concentration of zinc and alloying metals, but such temperature must be below the melting point of the alloys comprising the crusts desired to be removed.

The temperature may be maintained at the 65 bottom of kettle A somewhat above the eutec-

tic temperature of the bullion flowing therefrom and may be approximately the same as the top of kettle B, but the temperature at the bottom of kettle B is just above the eutectic temperature of the residual bullion.

In practice, however, it is desirable that the kettle B should be maintained at a higher temperature at the top than the outflow from the kettle A. By maintaining a higher temperature at the top of kettle B a 70 larger quantity of low grade crusts is maintained in circulation in B kettle, thereby ensuring a more consistent content of alloying metal in the residual bullion discharged from the bottom of the said kettle B.

It will be obvious that in operating with two kettles in series with the temperatures of the bottom of kettle A substantially the same as the top of kettle B the two kettles are performing the same functions as will 80 obtain in one kettle of dimensions equal to the combined depth of the two, the crusts formed in the lower part and cooler zone of the combined kettle being redissolved in the bullion in its upper part and hotter zone, 85 and these crusts will correspond in some degree with those crusts which would have been skimmed off from kettle B and regularly fed into the top of kettle A.

Consequently the invention may be conducted for the refining of bullion in one 90 kettle, the dimensions of such kettle being such as to ensure that the decreasing temperatures may be maintained from that at the top, which is below the melting point of 95 crusts desired to be removed, and sufficiently high to ensure the solution or absorption of the zinc added and the low grade crusts rising to the surface from the cooler zones, to that at the bottom which is just above the 100 eutectic temperature of the residual bullion delivered therefrom.

Instead of subjecting the top of the kettles or other apparatus in which the operation is conducted to external heat for the purpose of 110 obtaining the necessary temperature, I may preheat the bullion flowing into the kettle to such a degree as is necessary. Or alternatively I may preheat the bullion only to a limited extent with a view to reducing the 115 external heating of the top of the kettle.

In conducting the operation, therefore, it is preferable to preheat the bullion flowing into the kettle A in a small reverberatory furnace C and I have found in practice that 120 external heating of the kettles may be entirely dispensed with. By interposing a small reverberatory furnace immediately before the inflow into the kettles and causing the bullion to flow therethrough and be preheated therein to the necessary temperature 125 to ensure that the bullion has the required degree in the top of the kettles the operation may be conducted without any heating of the kettles. The maintenance of the decreasing 130

temperatures in the kettles to the temperature at the bottom just above the eutectic temperature of the residual bullion may be obtained by regulating the rate of flow of the bullion through the kettle or by subjecting the lower portions of the kettles to cooling means.

The invention therefore lends itself to an exceedingly simple arrangement of plant comprising a series of kettles G and H and small reverberatory furnaces C and D, the bullion being caused to flow continuously through from one reverberatory furnace C to a kettle and thence into another reverberatory furnace D from which it passes to the next kettle B in series, the regulation of the temperatures in the kettles being wholly or in part controlled by the temperatures in the said reverberatory furnaces C and D.

20 The following example will illustrate one application of this invention in which preferential removal of crusts relatively rich in gold is first obtained followed by the removal of crusts relatively rich in silver.

25 *Example.*—A crude bullion assaying approximately 60-ozs. silver, 100 grains gold per ton, and 0.1% copper was continuously preheated in a reverberatory furnace and fed into a kettle at the rate of 20 tons per hour, 30 together with an amount of zinc in regular additions equivalent to 10-lbs. per ton of bullion treated. The preheating of the bullion was such as to ensure a temperature at the top of the kettle of 500° C. and the temperature at the bottom of the kettle at 330° C. The residual bullion was continuously withdrawn from the bottom of the kettle by an overflow spout delivering just below the surface of the metal in the kettle and the 35 crusts accumulating on the surface of the kettle were skimmed off intermittently.

40 The residual bullion was found to assay 0.8 grains per ton gold and 55-ozs. per ton silver, whilst the crusts removed assayed 8-ozs. per ton gold and 200-ozs. per ton silver.

45 The residual bullion flowing from the above degolding treatment was then passed through another reverberatory furnace C for preheating and fed into kettle G of a series 50 of two kettles. The preheating in the reverberatory furnace C was such as to ensure a temperature of 450° C. at the top of kettle G and a temperature of 330° C. to 340° C. at the bottom thereof. The bullion delivered 55 from the bottom of kettle G was then passed through a further reverberatory furnace D and again preheated and fed to the top of kettle H. The temperature maintained in this last reverberatory furnace was such as 60 to ensure that the temperature at the top of kettle H was 450° C. and an amount of zinc equivalent to 16-lbs. per ton of bullion treated was regularly fed to the top of this kettle H. The temperature at the bottom of kettle H 65 was maintained at 330° C. Crusts accumu-

lating in the top of kettle H were skimmed from time to time and added regularly to the top of kettle G. The crusts accumulating in the top of kettle G were removed off from time to time and were found to assay 70 2000 ozs. silver per ton, whilst the residual bullion discharging from the bottom of kettle H assayed 0.15 ozs. silver per ton.

75 By the application of this invention the refining of bullion may be effected with a considerable saving in labor as compared with the operation of the "Parkes" process as hitherto practised. The continuous flow of the bullion through the kettles or other vessels employed dispenses with the labor incidental 80 to the cooling of the kettles as at present practised, and the transfer of bullion from one kettle to another. The arduous and laborious operation of scraping the kettles as required in the present operation of the 85 Parkes process is obviated. If the invention is operated in one kettle of suitable dimensions as described, the skimming of crusts from kettle B is entirely dispensed with, reducing the labor involved in the skimming 90 by over 50% as compared with the Parkes process as at present practiced with two zincings. In addition more consistent results can be obtained due to the fact that there is less dependence upon manual labor. Again, 95 by dispensing with the intermittent heating and cooling of the kettles and maintaining even temperatures upon the kettles during the flow of bullion therethrough, maintenance costs can be reduced due to less wear and tear and breakage of kettles, whilst a considerable saving in fuel can be effected. In addition a reduced plant is necessary for handling a given quantity of bullion, thereby effecting a considerable saving in capital 100 cost.

I claim:

1. In the continuous refining of lead bullion, incorporating with the bullion an amount of zinc sufficient for the formation of alloys of one or more of the alloying metals desired to be removed and a residual bullion relatively low in the said alloying metal or metals and subjecting the said bullion during its continuous flow to a decreasing range of temperatures the upper of which is sufficiently high for the solution or incorporation of the said zinc in the bullion and below the melting point of the alloy comprising the crusts to be removed, whilst the lower of such range is just above the eutectic temperature of the residual bullion desired to be produced, continuously withdrawing the residual bullion and continuously or intermittently removing the crusts accumulating.

2. In the continuous refining of lead bullion in one or more stages, incorporating with the bullion in each stage of an amount of zinc in the form of virgin zinc and/or

crusts sufficient for the formation of alloys of one or more of the alloying metals desired to be removed, and a residual bullion relatively low in the said alloying metal or metals, and subjecting the bullion in each stage during its continuous flow therethrough to a decreasing range of temperatures, the upper of which is sufficiently high for the solution or incorporation of the said zinc in the bullion but below the melting point of the alloy comprising the crust to be removed whilst the lower of such range in the last stage is just above the eutectic temperature of the residual bullion desired to be produced, continuously withdrawing the residual bullion from the last stage and continuously or intermittently removing the crusts accumulating in each stage.

3. In the continuous refining of lead bullion in one or more stages, incorporating with the bullion in each stage of an amount of zinc in the form of virgin zinc and/or crusts sufficient for the formation of alloys of one or more of the alloying metals desired to be removed, and a residual bullion relatively low in the said alloying metal or metals, and subjecting the bullion in each stage during its continuous flow therethrough to a decreasing range of temperatures, the upper of which is sufficiently high for the solution or incorporation of the said zinc in the bullion but below the melting point of the alloy comprising the crust to be removed whilst the lower of such range in the last stage is just above the eutectic temperature of the residual bullion desired to be produced, continuously withdrawing the residual bullion from the last stage and continuously or intermittently removing the crusts accumulating in each stage, and returning the crusts accumulating in the second or succeeding stages to a preceding stage.

4. In the continuous refining of lead bullion in one or more stages, incorporating with the bullion in each stage of an amount of zinc in the form of virgin zinc and/or crusts sufficient for the formation of alloys of one or more of the alloying metals desired to be removed, and a residual bullion relatively low in the said alloying metal or metals, and subjecting the bullion in each stage during its continuous flow therethrough to a decreasing range of temperatures, the upper of which is sufficiently high for the solution or incorporation of the said zinc in the bullion but below the melting point of the alloy comprising the crust to be removed whilst the lower of such range in the last stage is just above the eutectic temperature of the residual bullion desired to be produced, continuously withdrawing the residual bullion from the last stage and continuously or intermittently removing the crusts accumulating in each stage, preheating the bullion previous to any one stage to

such a degree as is necessary to maintain the requisite temperature in that stage.

5. In the continuous refining of lead bullion, incorporating with the bullion in one or more stages of an amount of zinc in the form of virgin zinc and/or crust necessary for the preferential formation of alloys of one or more of the alloying metals desired to be removed, and a residual bullion relatively low in such alloying metal or metals and subjecting the bullion in each stage to a decreasing range of temperatures, the upper of which is sufficiently high for the solution and incorporation of the said zinc whilst the lower of such range in the last stage is just above the eutectic temperature of the residual bullion relatively low in the said alloying metal or metals to be removed, continuously or intermittently removing the crusts accumulating in each stage and returning the crusts accumulating in the second and succeeding stages to a preceding stage, continuously withdrawing the said residual bullion, incorporating with the said residual bullion in one or more stages of an amount of zinc in the form of virgin zinc and/or crust for the formation of alloys of the remaining alloying metal or metals, and a residual bullion relatively low in such alloying metal or metals, and subjecting the bullion in each stage to a decreasing range of temperatures, the upper of which is sufficiently high for the solution and incorporation of the said zinc whilst the lower of such range in the last stage is just above the eutectic temperature of the residual bullion desired to be produced, withdrawing the said residual bullion continuously, and continuously or intermittently removing the crusts accumulating in each stage and returning the crusts accumulating in the second and succeeding stages to a preceding stage.

6. In the refining of lead bullion, feeding the bullion continuously through a kettle or series of kettles, incorporating with the bullion the necessary amount of zinc in the form of virgin zinc and/or crusts for the formation of alloys of one or more of the alloying metals desired to be removed and a residual bullion relatively low in the said alloying metal or metals, maintaining the bullion in the top of the said kettles or first kettle in the series at a temperature sufficiently high for the solution or incorporation of the said zinc in the bullion but below the melting point of the alloy comprising the crusts to be produced, maintaining the temperature of the bullion at the bottom of the kettle or last kettle in the series at a temperature just above the eutectic temperature of the residual bullion desired to be produced, continuously removing the residual bullion from the bottom of the kettle or last kettle in the series and continuously or

intermittently removing the crust accumulating.

7. In the refining of lead bullion, feeding the bullion continuously through a kettle together with the necessary amount of zinc for the formation of alloys of one or more of the alloying metals desired to be removed and a residual bullion relatively low in the said alloying metal or metals, maintaining 5 the bullion in the top of the said kettle at a temperature sufficiently high for the solution or incorporation of the said zinc in the bullion but below the melting point of the alloy comprising the crusts desired to be removed, maintaining the temperature of the 10 bullion at the bottom of the kettle just above the eutectic temperature of the residual bullion desired to be produced, withdrawing the residual bullion continuously from the bottom of the 15 said kettle and continuously or intermittently removing the crusts accumulating on the top of the said kettle.

8. In the refining of lead bullion, feeding the bullion continuously through a series of 20 two or more kettles together with the necessary amount of zinc in the form of virgin zinc and/or crusts for the formation of alloys of one or more of the alloying metals desired to be removed and a residual bullion relatively low in the said alloying metal or metals, maintaining the bullion at the top of the 25 first kettle in the series at a temperature sufficiently high for the solution or incorporation of the zinc in the bullion but below the melting point of the alloy comprising the crusts desired to be removed, maintaining the temperature of the 30 bullion at the bottom of the last kettle in the series just above the eutectic temperature of the residual bullion to be produced, feeding the crusts accumulating on the surface of the second and succeeding kettles into the top of a preceding kettle, withdrawing the residual bullion continuously from the bottom of the 35 last kettle in the series and continuously or intermittently removing the crusts accumulating on the top of the first kettle.

9. In the refining of lead bullion, feeding the bullion continuously through a kettle or 40 series of kettles, incorporating with the bullion the necessary amount of zinc in the form of virgin zinc and/or crusts for the formation of alloys of one or more of the alloying metals desired to be removed and a residual bullion relatively low in the said alloying metal or metals, preheating the said bullion in a reverberatory or other suitable furnace to such a temperature as is necessary for 45 maintaining the bullion in the top of the kettle or the first kettle in the series at a temperature sufficiently high for the solution or incorporation of the said zinc in the bullion but below the melting point of the alloy comprising the crusts desired to be removed, maintaining the temperature of the 50 bullion during its passage through the first series of kettles at a temperature just above the eutectic temperature of the residual bullion relatively low in the said alloying metal or metals to be preferentially removed, continuously discharging the residual bullion into the succeeding series incorporating with the bullion during its passage through the 55

at the bottom of the kettle or the last kettle in the series at a temperature just above the eutectic temperature of the residual bullion desired to be produced, withdrawing the residual bullion continuously from the bottom of the said kettle or the last kettle in the series and continuously or intermittently removing the crusts accumulating on the top of the said kettle.

10. In the refining of lead bullion, feeding the bullion continuously through a series of two or more kettles, incorporating with the bullion the necessary amount of zinc in the form of virgin zinc and/or crusts for the formation of alloys of one or more of the alloying metals desired to be removed and a residual bullion relatively low in the said alloying metal or metals, preheating the said bullion in a reverberatory or other furnace prior to the said bullion being delivered into the top of each of the said kettles in the series whereby the temperature of the bullion is raised therein during its passage to such a degree as is necessary for maintaining the bullion in the top of each of the said kettles at a temperature sufficiently high for the solution or incorporation of the zinc either as virgin zinc or in the form of low grade crusts in the bullion, but below the melting point of the alloy comprising the crusts desired to be removed, maintaining the temperature of the bullion at the bottom of the last kettle in the series just above the eutectic temperature of the residual bullion desired to be produced, feeding the crusts accumulating on the surface of the second or succeeding kettles into the top of a preceding kettle, withdrawing the residual bullion continuously from the bottom of the last kettle in the series and continuously or intermittently removing the crusts accumulating on the top of the said kettle.

11. In the refining of lead bullion, feeding the bullion continuously through two or more series of kettles, incorporating with the bullion during its passage through the first series the necessary amount of zinc in the form of virgin zinc and/or crusts for the preferential formation of alloys of one or more of the alloying metals and a residual bullion relatively low in such alloying metal or metals maintaining the bullion at the top of the first kettle of the first series at a temperature sufficiently high for the solution or incorporation of the said zinc in the bullion, but below the melting point of the alloy comprising the crusts to be removed, maintaining the temperature of the bullion at the bottom of the said last kettle of the first series just below the eutectic temperature of the residual bullion relatively low in the said alloying metal or metals to be preferentially removed, continuously discharging the residual bullion into the succeeding series incorporating with the bullion during its passage through the 110

- said succeeding series the necessary amount of zinc in the form of virgin zinc and/or crusts for the formation of alloys of the remaining alloying metal or metals desired to be removed and obtaining a residual bullion relatively low in the said alloying metal or metals, maintaining the bullion at the top of the first kettle of the said succeeding series at a temperature sufficiently high for the solution or incorporation of the zinc in the bullion but below the melting point of the alloy comprising the crusts desired to be removed, maintaining the temperature of the bullion at the bottom of the last kettle just above the eutectic temperature of the residual bullion desired to be produced and relatively low in such alloying metals, withdrawing the said residual bullion continuously from the bottom of the last kettle and continuously or intermittently removing the crusts accumulating in the said succeeding series of kettles relatively high in the said remaining alloying metal or metals. 12. In the refining of lead bullion, feeding the bullion into a reverberatory or other suitable furnace for preheating it to the required temperature and discharging the said preheated bullion into the top of the first of two series of kettles, together with the necessary amount of zinc for the formation of alloys in the form of crusts relatively rich in one or more of the alloying metals (such as gold) and obtaining a residual bullion relatively low in the said alloying metal or metals continuously passing the said bullion through the first series of kettles and discharging the same continuously from the bottom of the last kettle in the first series at a temperature just above the eutectic temperature of the residual bullion relatively low in the said alloying metal or metals, continuously or intermittently removing the crusts relatively rich in such alloying metal or metals from the top of the first kettle, in the first series, feeding the bullion to a reverberatory or other suitable furnace in which it is preheated to the desired temperature and then feeding the same continuously through the second series of kettles, feeding an amount of zinc into the first kettle of the second series sufficient for the formation of alloys in the form of crusts relatively high in the remaining alloying metal or metals and obtaining a residual bullion relatively low in the said alloying metal or metals, maintaining the temperature of the bullion at the bottom of the first kettle of the second series somewhat above the eutectic temperature of the bullion, continuously discharging therefrom, feeding the said bullion into a reverberatory or other suitable furnace for preheating it and then discharging the same into the second kettle of the second series, feeding the crusts accumulating on the surface of the second kettle of the second series into the top of the first kettle of the second series, withdrawing the residual bullion continuously from the bottom of the second kettle in the second series relatively low in the said alloying metal or metals and continuously or intermittently removing the crusts accumulating in the top of the first kettle of the second series relatively high in the said alloying metal or metals. In witness whereof I hereunto affix my signature. 75  
GEORGE KENNETH WILLIAMS. 80  
85  
90  
95  
100  
105  
110  
115  
120  
125  
130